

## UNITED STATES PATENT OFFICE

2,081,176

## FUEL OIL

Amiot P. Hewlett, Cranford, and Charles H. Cole,  
Roselle Park, N. J., assignors to Standard Oil  
Development Company, a corporation of Delaware

No Drawing. Application December 30, 1933,  
Serial No. 704,786

## 11 Claims.

(Cl. 44—8)

This invention relates to fuel oils and methods of preparing same or of reducing the combustion residues of same.

When fuel oils are burned, a small amount of carbonaceous residue or "coke" results from the combustion. The formation of this residue is a disadvantage, for instance, in leading to the clogging of the burners through which the fuel oil is fed. As a result it makes necessary the shutting down of the burner occasionally to remove the residue and it may also at more frequent intervals necessitate a readjustment of the burners in order to compensate for the reduced amount of fuel oil being fed through the burners.

It is an object of the present invention to avoid these and other difficulties by greatly reducing the amount of this carbonaceous residue or coke.

According to this invention, it has been found that the addition of a relatively small quantity of a high boiling substance to a domestic fuel oil results in a decrease in the quantity of the carbonaceous residue formed during burning.

The fuel oils which may be treated in accordance with this invention may have properties varying over a relatively wide range but the invention is particularly applicable to fuel oils having a Saybolt viscosity of less than 45 seconds at 100° F. It also applies to even lighter fuel oils, for example, those having a viscosity of 35 seconds or even considerably less at 100° F. even including kerosene generally considered to have an A. P. I. gravity of 41 to 45° and other light range oils. Typical fuel oils on the market which can be used are:

|                           | Gravity<br>A. P. I. | Average viscosity at 100° F.<br>(Saybolt) |
|---------------------------|---------------------|-------------------------------------------|
| Domestic light fuel oil   | 36 minimum.         | Less than 35.                             |
| Domestic medium fuel oil  | 28 minimum.         | About 35.                                 |
| Domestic heavy fuel oil   | About 24-26.        | About 41 or 42.                           |
| Light industrial fuel oil | 18-22.              | 40-75.                                    |

The source of crude from which these oils may be derived is not material. They may be so-called native oils, i. e., obtained by mere distillation from the original crude oil or else they may be obtained by cracking of a crude or some fraction thereof. The original oil, from which the heating oil is obtained, may be of paraffinic, naphthenic or mixed type; the fuel oil may also be derived from coal, shale and other carbonaceous materials by distillation, destructive distillation, hydrogenation, etc.

The high boiling substance to be added according to the present invention should preferably have a mid-boiling point slightly higher than the end point of the heating oil to which it is to be added (which is generally about 550

to 600° F.). In other words, the addition agent should have a boiling point (or mid-boiling point between the approximate limits of 600° and 700° or 750° F. It should also be a fraction having a Saybolt viscosity between the approximate limits of 40 and 500 seconds at 100° F. A wide variety of types of substances may be used as the addition agent, for instance, high boiling mineral oils or organic compounds such as hydrocarbons, esters, alcohols, ketones, etc. or chlorinated or other derivatives thereof. This addition agent also preferably has a relatively high solvent power (such as a kauri butanol value above about 15) or gum fluxing action (which means capable of preventing precipitation of other substances although not capable of actually dissolving them after they are once precipitated); and between oils or other substances having equal characteristics in other respects it is preferable to use the one having the lower Conradson carbon. The kauri butanol test is described in circular 378 (February, 1931) of the American Paint and Varnish Manufacturers Association. The naphthenic type of oils and other hydrocarbons described and claimed in co-pending application Ser. No. 658,153 of Sloane and Wasson, as well as the high boiling esters and other oxygenated organic compounds described and claimed in co-pending application Ser. No. 667,039 of Jones I. Wasson are suitable for use according to the present invention. Although the addition agent should have a boiling point higher than that of the fuel oil to which it is added still it should not be too high boiling or too viscous. For instance, the addition of 1% of a viscous Pennsylvania cylinder stock to a fuel oil actually caused a slight increase in the coke residue formed on combustion. If a petroleum oil is used as addition agent, it is preferably an overhead product; in other words, it should be obtained by distillation, although fractions of suitable gravity and viscosity may be separated from a crude or residual stock by extraction, fractional precipitation or in any other desired manner.

The amount of the addition agent to be used is preferably between the approximate limits of 0.5 and 1.5%. Satisfactory results have been obtained with 0.75 and with 1.0%, although it is obvious that lesser and greater amounts, for instance, between the approximate limits of 0.1 and 5.0% may be used under certain circumstances. In general, the amount to be used depends upon the type of the oil treated as well as the type of addition agent and the type of burner in which the fuel oil is to be used. The invention has been found particularly applicable to fuel oils to be used in the Timken and other types of rotary burners.

In carrying out the invention, the desired

amount (measured by either weight or volume) of addition agent, such as one of the high boiling oils or organic compounds mentioned above, is incorporated into the larger bulk of fuel oil 5 with sufficient agitation to insure thorough mixing. If desired, heat may be used to facilitate thorough solution. This high boiling substance may be added any time prior to actual burning. If added prior to storage it may present the additional advantage of helping to stabilize the fuel oil during storage.

The valuable results obtained by the application 10 of this invention include primarily a reduction in the amount of carbonaceous or coke residue obtained upon combustion of the fuel oil, although in some instances there is also an additional advantage in having a better distribution of the coke residue which is left. This latter feature is of more importance for range oils than it is 15 for fuel oils to be used in furnaces. The reasons for the great reduction in the amount of carbonaceous residue and other advantages of the invention are not well understood but it is believed that the presence of the small amount of 20 the high boiling addition agent prevents the precipitation of the coke or carbonaceous material which would otherwise tend to precipitate and hence it maintains a more uniform or homogeneous solution longer and at higher temperatures 25 than does the fuel oil alone. It thus facilitates combustion of the entire mass.

The coking test which has been found satisfactory for comparing the amount of carbonaceous residue obtained on combustion of a fuel oil is 30 carried out by dropping 100 cc. of the fuel oil slowly (at the rate of about 100 cc. per hour) drop by drop into an iron dish which is maintained at 700° F. The increase in weight of the dish before and after the test represents the 35 amount of carbonaceous residue or coke obtained from the combustion of 100 cc. of the fuel oil.

Although it is not intended that the invention be limited thereby, the following examples are given to illustrate the invention:

| Example number                                                   | Addition agent |                             | Coke residue, mg./100 cc. oil |
|------------------------------------------------------------------|----------------|-----------------------------|-------------------------------|
|                                                                  | Vis., 100° F.  | B. Pt. or (Mid B. Pt.), °F. |                               |
| 50                                                               |                |                             |                               |
| 1. Fuel oil A<br>Ditto+1% Colombian pale oil                     |                | 300                         | 91<br>22                      |
| 2. Fuel oil B (end pt.=582° F.)<br>Ditto+1/4% Colombian pale oil |                | 300                         | 228<br>108                    |
| 3. Oil B+1/4% Penna. Lube Dist., narrow cut (500-700° F.)        | 60             | About 650                   | 38                            |
| 4. Oil B+1/4% octadecyl naphthalene                              | 113            | About 700                   | 117                           |
| 5. Oil B+1/4% octadecyl benzol                                   | 58             | About 650                   | 92                            |
| 6. Oil B+1/4% methyl oleate                                      |                | About 520                   | 184                           |
| 7. Oil B+1/4% amyl stearate                                      | About 50       | About 600                   | 55                            |

The exact theory of operation of the invention is not well understood and it is therefore desired that the invention should not be limited to any 65 particular theories nor to the examples which are

given merely for the sake of illustration. In the appended claims it is intended to claim all inherent novelty in the invention as broadly as the prior art permits.

We claim:

1. A fuel oil of less than 40 seconds viscosity Saybolt at 100° F. forming a high carbon residue, containing from 0.1 to 5.0% of an added soluble hydrocarbon, liquid at ordinary temperature, of substantially higher boiling point than said fuel oil and also having a kauri butanol solvent power above about 15, said soluble hydrocarbon being capable of reducing the coke residue of the fuel oil.

2. A fuel oil composition according to claim 1 in which the added soluble hydrocarbon is a petroleum distillate.

3. A fuel oil of less than 40 seconds viscosity Saybolt at 100° F. and having a gravity of 18 to 36° A. P. I., forming a high carbon residue, and containing from 0.1 to 5.0% of an added soluble liquid having a boiling point higher than the end-point of the fuel oil and having a kauri butanol solvent power above about 15, said liquid being capable of reducing the coke residue of the fuel oil.

4. A fuel oil composition according to claim 3 in which the added liquid is of petroleum origin.

5. A fuel oil composition according to claim 3 in which the added liquid is a distillate of a naphthenic type petroleum oil.

6. A fuel oil composition according to claim 3 in which the added liquid has a viscosity between 40 and 500 seconds Saybolt at 100° F.

7. A domestic fuel oil forming a high carbon residue, comprising a major proportion of an oil having a Saybolt viscosity of less than about 45 seconds at 100° F. and a distillation end point of about 550 to 600° F., and about 0.75 to 1.0% of a pale oil having a mid-boiling point between the approximate limits of 600 and 700° F.

8. The method of preparing a domestic fuel oil, which comprises adding about 0.1% to 5.0% of a pale oil having a mid-boiling point between the approximate limits of 600 and 700° F. to a fuel oil having a Saybolt viscosity of less than about 45 seconds at 100° F. and a distillation end point of about 550 to 600° F. whereby the amount of carbonaceous residue resulting from the combustion of the fuel oil is reduced.

9. The method of reducing the amount of carbonaceous residue or coke resulting from the combustion of a fuel oil of less than 40 seconds viscosity Saybolt at 100° F., which comprises adding thereto from 0.1% to 5.0% of soluble hydrocarbon, liquid at ordinary temperatures, of substantially higher boiling point than said fuel oil and also having a kauri butanol solvent power above about 15.

10. A fuel oil composition according to claim 3 in which the added liquid is an oxygenated organic compound.

11. A fuel oil composition according to claim 3 in which the added liquid is an ester of a monohydric alcohol.

AMIOT P. HEWLETT,  
CHARLES H. COLE.